

## UNITED STATES PATENT OFFICE.

FREDERICK KAYE, OF ASHTON-ON-MERSEY, ENGLAND.

## PAPER MAKING.

No Drawing.

Application filed June 22, 1921. Serial No. 479,642.

*To all whom it may concern:*

Be it known that I, FREDERICK KAYE, a subject of the King of Great Britain and Ireland, residing at Ashton-on-Mersey, in the county of Chester, England, have invented new and useful Improvements Relating to Paper Making, for which I have filed application for patent in Great Britain June 25, 1920, No. 17,252, and of which the following is a specification.

This invention refers to the manufacture of paper and paper-like materials, and its chief object is the production of paper or the like which is remarkably strong both with regard to tensile strength and to resistance to abrasion and to repeated bending while under tension. Another object is a paper or the like which has a considerable bursting strength. A further object is a paper or the like in which low grade fibres may be profitably used.

According to the invention, any natural india-rubber-containing latex, or any india-rubber-containing latex preserved by ammonia, formaldehyde and the like, or any gutta-containing latex, or balata-containing latex, singly or combined, is or are added to the usual paper making materials, cotton, jute, linen hemp, wood pulp or other vegetable or animal fibres, as well as mineral fibres such as asbestos, together with any mineral fillers, such as china clay and the like.

The said latex or latices is or are added to the paper pulp after the latter has been beaten to the required extent for the quality of paper aimed at and the quantity of latex or latices added is in proportion to the quality of the paper to be made and the nature of the fibres, and other materials used in the composition of the paper. After thoroughly mixing the latex or latices with the pulp, which may be done in the beater, a coagulative agent is added, said agent being added according to the nature and state of the latex, and being such as acetic acid, formic-acid or any other suitable organic or mineral acid, or small quantities of mineral salts.

When a satisfactory coagulation has been effected the contents of the beater are transferred to the cistern or pulp-holding tank of the usual paper making machine and run through the machine in the ordinary manner. The paper may be sized in the usual

manner, before or after the addition of the rubber, gutta, or balata-containing latices.

The dried paper can afterwards be vulcanized by any suitable process.

The india rubber content of the latex used having been determined in some well-known manner, the volume of latex required for a known weight of pulp can be taken and suitably diluted before addition to the beaten pulp. The dilution should be considerable, say 1% to 0.1%, or even less of rubber, gutta or balata content. The amount of coagulative agent should be the minimum quantity necessary which can be experimentally determined.

The nature and quantity of coagulative agent may vary with the nature and character of the latex or latices employed, but such will be easily determined by those skilled in the art.

Highly satisfactory paper has been manufactured by this process, using the latex of *Hevea brasiliensis*, and containing 0.5%, 1%, 2%, 4% and 5% of rubber to the weight of dried paper, whilst much more resinous latices have been successfully used to produce papers for special purposes containing as much as 10% of coagulative material.

Paper containing india-rubber has a high tensile strength. The folding number, as determined by the Schopper folding machine, of samples of paper containing 0.5% of rubber and vulcanized, has reached 5,000 to 6,000. Without vulcanization, paper containing 2% of rubber often has a folding number of 2,000 and over.

The bursting strength of many papers made from chemical wood pulp containing rubber from the latex of *Hevea brasiliensis*, or from the coagulum of highly resinous latices containing rubber, gutta or balata, is equal to that of paper made by the "Kraft" process.

The quality of paper being improved by this process the time of beating may, in many cases, be considerably shortened, thus reducing the cost of manufacture. Further, by this invention fibres of low grade can be profitably used for the purpose of paper making. The invention may be usefully applied in the making of mill board and similar paper-like materials.

What I claim is:—

1. The process of making paper, which consists in adding to the paper pulp after

digestion and prior to passing the pulp through a paper-making machine, a rubber-containing latex, mixing the mass thereby to disseminate the latex between the particles of pulp, and passing the mixed mass through a paper-making machine.

2. The process of making paper, which consists in adding to the paper pulp a rubber-containing latex, mixing the mass thereby to disseminate the latex between the particles of the pulp, passing the mixed mass through a paper-making machine, and vulcanizing the resulting paper.

3. The process of making paper of any desired thickness consisting in adding to the ordinary materials used in making paper, after such materials have been beaten, rubber-containing latex, gutta-containing latex, or balata-containing latex, or a combination of any two of these latices mixing the said materials and latex or latices together, adding a coagulative agent to the mixture, and after suitable coagulation, passing the mixture through a paper-making machine, as set forth.

4. In a process of making paper of any desired thickness adding to the paper pulp, after being beaten, rubber-containing latex, gutta-containing latex, or balata-containing latex diluted to contain only a small content of rubber, gutta or balata relatively to

the weight of paper to be produced, mixing the pulp and diluted latex, adding a coagulative agent to the mixture, and after suitable coagulation, passing the mixture through a paper-making machine, as set forth.

5. In a process of making paper of any desired thickness adding to the paper pulp after being beaten, rubber-containing, gutta-containing, and balata-containing latices mixed with each other in suitable proportions, mixing the beaten materials and latices together, adding a coagulative agent to the mixture, and after coagulation passing through a paper-making machine, substantially as herein set forth.

6. The process of making paper of any desired thickness consisting in adding to the ordinary materials used in making paper, after the materials have been beaten, rubber-containing latex, gutta-containing latex, or balata-containing latex, mixing said materials and latex together, adding a coagulative agent to the mixture, and after suitable coagulation, passing the mixture through a paper-making machine, and finally vulcanizing the paper, as set forth.

In testimony whereof I have signed my name to this specification.

FREDERICK KAYE.